

## UNITED STATES PATENT OFFICE

2,131,146

TREATMENT OF MATERIALS FOR VARYING  
THEIR AFFINITY

Paul Schlack, Berlin-Treptow, Germany, assignor to I. G. Farbenindustrie Aktiengesellschaft, Frankfort-on-the-Main, Germany, a corporation of Germany

No Drawing. Application December 5, 1935, Serial No. 53,004. In Germany December 8, 1934

## 14 Claims.

(Cl. 8—5)

This invention relates to a treatment of materials for varying their affinity.

One of its objects is a process of treating materials for varying their affinity. Another object is the material obtained by this process. Further objects will be seen from the detailed specification following hereinafter.

According to the present invention it has been found that the chemical behavior of natural or artificial products from proteins or of materials containing or consisting of highly molecular materials which are not proteins but contain basic nitrogen, towards dyestuffs can be considerably changed if they are treated with an alkylating agent selected from the group consisting of esters and diazoparaffins, for instance, with a reactive alkylester of a mineral acid or a mixed organic-inorganic acid as for instance alkyl- or aryl-sulfonic acid. In this case apparently alkylated products are formed the electrochemical character of which is different from that of the starting materials. The alkylation takes place at the nitrogen atom, however, a change of the electrochemical character is also effected by alkylation of carboxyl groups, as for instance in the case of wool. Alkylating agents of this kind are for instance, ethyliodide, ethylbromide, n-butyliodide, ethylenechlorhydrine, benzylchloride, p-nitrobenzylchloride, chloracetic methylester, chloroacetone, chloracetaldehyde, dialkylsulfate, alkylsulfonic acid alkylesters, the sodium salt of chloromethylbenzene sulfonic acid, the sodium salt of a xylol sulfonic acid halogenated in the side chain, toluene sulfonic acid alkylesters, naphthalene sulfonic acid alkyl esters, salts of carboxyaryl sulfonic acid alkyl esters, trichloroxypropylamine hydrochloride,  $\beta$ -tris- $\beta$ -chlorethyl-aminehydrochloride and tetrachloroxypropyl ammonium chloride, diazo paraffins such as diazomethane or diazoethane.

The extent to which the material is changed is mainly dependent upon three factors, namely, the swelling condition of the material, the reactivity of the agent and the temperature. The conditions of reaction under which for instance, a sufficient coloring effect is obtained may therefore vary widely. Apart from the fact that from case to case the demands vary for instance, according to whether a relatively slight improvement of the dyeing capacity is desired particularly when working in a neutral bath or whether a strong coloring contrast is desired. In the case of wool and other animal fibers preferably a temperature of at least 40° C. is applied when working in non-aqueous solutions, since with this tem-

perature the reactivity of the material begins to increase.

If for special reasons it is desired to work at a temperature lower than 40° C. it is necessary to prolong the period of reaction. In this case advantageously easily reacting alkylating agents are used, for instance, an alkyl iodide. In any case, a boiling of dry wool with ethylbromide for two hours gives no effect. Also when imparting a stronger reactivity to wool by exposing it to the influence of an atmosphere containing 60 per cent of relative moisture the influence is only very slight and practically without value as experiments have shown. A reaction period of at least 3 hours is necessary for the production of a material which has clearly a greater affinity to acid dyestuff than the nontreated material. Also when treating wool with dimethylsulfate in an alkaline medium at room temperature no useful effect is obtained if the alkylating agent is not finely dispersed or emulsified in the aqueous medium. However, an effect is produced if wool is boiled in methanol in the presence of 10 or 20 per cent of dimethylsulfate whereby the addition of an acid binding agent facilitates the reaction. In the same manner a strong effect is produced if wool is treated with an aryl sulfonic acid alkyl ester in an aqueous suspension in the presence of an acid binding agent such as prepared chalk.

The behavior towards dyestuffs of the objects treated is more or less profoundly changed; in particular the adsorptive capacity and the speed of fixation of the dyestuffs, dyestuff-derivatives, dyestuff components and other treating agents having acid groups, are generally considerably enhanced, while in the case of basic dyestuffs the reverse effect occurs. When the alkylating agent contains acid groups the foregoing relationships may be reversed.

The treatment forming the subject-matter of the invention may be applied at ordinary or raised temperature, the limits depending on the reactivity of the alkylating agent and the resistance of the goods under treatment. The speed of the reaction may also be influenced by the moisture in the atmosphere or in the goods under treatment. In the case of halogen compounds which react slowly, the chemical change can be hastened by a small addition of an iodide, for example, potassium iodide, tetramethyl ammonium iodide or trimethyldodecylammonium iodide. As already mentioned, the process may also be conducted in the presence of a neutral or alkaline acid binding agent, for example in the presence

of potassium acetate, borax, sodium phosphate, sodium silicate or of amines which are alkylated with difficulty. A particularly strong effect is obtained when the treatment is conducted with reactive esters of organic acids in the presence of alkylene oxides or their analogues, for example propylene oxide or epichlorhydrin. There may also be present in the process additions of other reactive materials named in U. S. patent application Ser. No. 40,352 filed September 12, 1935. Furthermore, agents capable of protecting the fiber, oxidizing or reducing bleaching agents and swelling agents such as formamide, thiourea, magnesium thiocyanate, zinc thiocyanate and methanol may be present. The alkylating agents may be used in the process as such or be produced or liberated in the presence of the goods to be treated, for example by thermal decomposition of labile alkyl halides or salts of imine-ethers, or nitroalkylurethanes.

The action of the alkylating agent can be combined with a drying or printing operation. Also an after-treatment of a finished dyeing may be advantageous for the purpose of improving the fastness thereof. In both cases it is obvious that the dyestuff must not be essentially changed by the alkylating agent. The fiber may be pre-treated before the alkylating operation with materials other than dyestuffs, for example with mordants, tanning agents, loading agents or insecticides. The after-treatment of finished colorings with alkylating agents is of particular importance, because in this manner an increased fastness is obtained. In both cases it must be considered that the shade of some dyes is changed. By changing the pH value of the substrate a changing of the shade of the coloring may be prevented or lessened. The changing of the coloring increases generally with an increasing pH value. Substances which are sufficiently volatile at low or moderate temperature and, if desired, under diminished pressure, are advantageously applied to the goods in the form of vapor in the manner described in my co-pending application Ser. No. 46,445 filed October 23, 1935.

The increase of the affinity or the speed of adsorption exhibited by the fibers or objects for certain groups of dyestuffs which follows the application of the invention is of particular importance in printing and in dyeing mixed fabrics or mixed yarns, for instance mixed yarns of wool and cellulose fibers or of wool and acetyl-cellulose fibers, particularly when the dyeing is to be conducted under feebly acid or neutral conditions at the lowest possible temperature.

The following examples illustrate the invention, the parts being by weight unless stated otherwise, and the parts by weight and parts by volume bearing the relationship to each other as that of the kilo to the liter:

*Example 1.*—1.7 parts of wool are heated at 80° C. for 14 hours in 1000 parts by volume of air containing 0.5 part of vapor of ethyl bromide and having a moisture saturation of 75 per cent. The wool, which is externally altered only to an unessential extent, adsorbs Alizarine Direct Blue A or Orange II (each 2 per cent.) in a neutral liquor much more strongly than wool which has not been treated and is dyed in the same dye-bath. The dyeings are also faster to washing than equally deep dyeings on untreated wool. The same dyeing differences are observed if the wool is soaped before dyeing.

75 Orange II (Schultz, 7th edition, Vol. I, page 86).

Alizarine Direct Blue A (Schultz, Vol. II, page 9, 7th edition).

*Example 2.*—Instead of the ethyl bromide prescribed in the foregoing example, chloracetic acid-ethyl-ester is similarly used, the duration of the operation being 16 hours at 70° C. and under a moisture saturation of 75 per cent. The above-named dyestuffs are adsorbed by the material at an essentially lower temperature than by normal wool.

*Example 3.*—Wool is impregnated with a solution of sodium benzyl-chloride-sulphonate of 10 per cent. strength containing  $\frac{1}{10}$  mol. of potassium iodide, calculated on the benzyl-chloride-sulphonate. The wool is then centrifuged and heated for 16 hours at 70° C. Acid dyestuffs, for instance Alizarine Direct Blue A, are more quickly fixed by the treated material than by ordinary wool.

*Example 4.*—Wool is heated for 16 hours at 80° C. in an atmosphere of 75 per cent. moisture saturation and containing benzyl chloride amounting to 20 per cent. of the weight of the wool. The treated skein is still pure white. When dyed with Alizarine Direct Blue A the dye is strongly adsorbed by the treated material already at 60° C. Even after an intermediate treatment with ammonia, the same relative difference exists.

*Example 5.*—Wool dyed with 2 per cent. of Orange II is treated for 16 hours at 50° C. in an atmosphere of 75 per cent. moisture saturation with ethyl iodide vapor. The fastness to washing is considerably improved. In like manner the fastness to washing of a 2 per cent. dyeing of Azofuchsin G on wool may be enhanced.

*Example 6.*—Wool is impregnated with an n/5-solution of tetrachlorhydroxypropylammonium chloride obtainable according to U. S. patent application Ser. No. 53,003 filed December 5, 1935 (cf. British Patent No. 454,320); and after having been centrifuged is heated for 16 hours at 80° C. After thorough washing, the treated wool is more powerfully dyed by means of Alizarine Direct Blue A than an untreated comparative sample.

*Example 7.*—Fibroin artificial silk is heated for 16 hours at 80° C. in an atmosphere of moisture saturation of 75 per cent. in the presence of ethyl iodide vapor. The treated artificial silk is dyed with Orange II not inconsiderably darker tints than untreated artificial silk in the same bath.

*Example 8.*—An acetate artificial silk containing a basic artificial resin of the polyvinyl series (content of basic tertiary nitrogen in the fiber being 0.4 per cent.) is dyed with 2 per cent. of Alizarine Direct Blue A in the presence of acetic acid. The dyed material is suspended for 14 hours in an atmosphere of 80 per cent. moisture saturation containing ethyl iodide vapor. The fastness to washing of the dyeing is not inconsiderably improved.

*Example 9.*—Zephir yarn is dyed in the usual manner with 3 per cent. of Amidonaphthol-Red BB (Schultz Farbstofftabellen 7th ed. suppl. vol. 65 page 8, No. 110) and is then heated for 12 hours with 8 per cent of propylene oxide and 20 per cent of ethyl iodide in an atmosphere containing about 92 per cent of relative moisture in a closed vessel of 100 parts of volume at 50° C. The after-treated wool can be washed at 80° C. without material change in the color and without bleeding on white material washed simultaneously. The non-after-treated coloring is removed to the greater part when washed under the same condi-

tions. In this case the white material is strongly colored.

Example 10.—10 parts of zephir yarn are treated with an aqueous dispersion of 5 parts of prepared chalk and 5 parts of toluenesulfonic acid methylester both being dispersed with 20 per cent of oleylpolyglycol, for 1 hour at 65° C. and for 1 hour at 75° C. in a bath containing 20 parts of liquid on one part of yarn. Then the yarn is thoroughly washed and treated with a soap solution. The treated wool is dyed more intensely with an acid dye, for instance, with Alizarine Direct Blue A (Schultz Farbstofftab. 7th ed. Vol. II, page 9) than the starting material.

Example 11.—Zephir-wool is treated with 15 per cent of ethyl bromide and 10 per cent of 1,2-propylene sulfide for 14 hours at 50° C. in an atmosphere with 75 per cent of relative moisture. The wool shows an appreciable improvement of the capacity of being dyed, particularly in a neutral bath. The colorings for instance, with Amidonaphthol-Red BB (Schultz Farbstofftab. 7th ed. suppl. vol., page 8, No. 110) are faster to water and washing than those of the untreated wool.

Example 12.—Wool is treated with an aqueous dispersion of 20 per cent of dimethylsulfate and 20 per cent of prepared chalk made with the aid of oleyl-polyglycol, for 2 hours at 40° C. in a bath containing 20 parts of treating liquid on 1 part of material to be treated. The thoroughly washed material is, in a neutral bath, dyed by means of acid dyes, for instance, of Orange II much more intensely than untreated material dyed in the same bath. Rinsing with a cold solution of ammonia before dyeing will not make the pretreatment ineffective. If a material is dyed which contains treated and untreated material, strong two-color effects are obtained.

40 What I claim is:

1. A process of increasing the affinity for acid dyestuffs of wool, natural silk, leather, artificial fibers containing a basic artificial resin, and artificial fibers containing a basic cellulose derivative, which comprises subjecting the material to the action of an alkylating agent selected from the group consisting of reactive alkyl esters and diazoparaffines.

2. A process of increasing the affinity for acid dyestuffs of natural and artificial organic products containing a quaternary amino group, together with a carboxyl group, combined in molecules of high molecular weight, which comprises subjecting the material to the action of an alkylating agent selected from the group consisting of reactive alkyl esters and diazoparaffines.

3. A process of increasing the affinity for acid dyestuffs of wool, natural silk, leather, artificial fibers containing a basic artificial resin, and artificial fibers containing a basic cellulose derivative, which comprises subjecting the material to the action of a reactive alkyl ester.

4. A process of increasing the affinity for acid dyestuffs of wool, natural silk, leather, artificial fibers containing a basic artificial resin, and artificial fibers containing a basic cellulose derivative, which comprises subjecting the material to the action of a diazoparaffine.

5. A process of increasing the affinity for acid dyestuffs of wool, natural silk, leather, artificial fibers containing a basic artificial resin, and artificial fibers containing a basic cellulose derivative, which comprises subjecting the material to the action of an alkylating agent selected from the group consisting of reactive alkyl esters and diazoparaffines in the presence of a compound selected from the group consisting of alkylene oxides, alkylene sulfides and alkylene imines. 10

6. A process of increasing the affinity for acid dyestuffs of wool, natural silk, leather, artificial fibers containing a basic artificial resin, and artificial fibers containing a basic cellulose derivative, which comprises subjecting the material to the action of an alkylating agent selected from the group consisting of reactive alkyl esters and diazoparaffines in the presence of a swelling agent. 15

7. A process of increasing the affinity to acid dyestuffs of wool, natural silk, leather, artificial fibers containing a basic artificial resin, and artificial fibers containing a basic cellulose derivative, which comprises subjecting the material to the action of an alkylating agent selected from the group consisting of reactive alkyl esters and diazoparaffines, and subsequently dyeing the material with an acid dyestuff. 20

8. A process of increasing the affinity to acid dyestuffs of wool, natural silk, leather, artificial fibers containing a basic artificial resin, and artificial fibers containing a basic cellulose derivative, which comprises subjecting the material to the action of an alkylating agent selected from the group consisting of reactive alkyl esters and diazoparaffines, and simultaneously dyeing the material with an acid dyestuff. 25

9. A process of increasing the affinity to acid dyestuffs of wool, natural silk, leather, artificial fibers containing a basic artificial resin, and artificial fibers containing a basic cellulose derivative, which comprises dyeing the material with an acid dyestuff, and subjecting it to the action of an alkylating agent selected from the group consisting of reactive alkyl esters and diazoparaffines. 30

10. An article comprising one of the group of materials consisting of wool, natural silk, leather, artificial fibers containing a basic artificial resin, and artificial fibers containing a basic cellulose derivative, said materials being substituted by alkyl radicals and having a substantially increased affinity for acid dyes. 35

11. Wool having a substantially increased affinity for acid dyestuffs, the molecule of said wool being substituted by an alkyl group. 40

12. Cellulose fibers having a substantially increased affinity for acid dyestuffs, said cellulose fibers having incorporated a basic artificial resin substituted by alkyl radicals. 45

13. Acetyl cellulose fibers having a substantially increased affinity for acid dyestuffs, said acetyl cellulose fibers having incorporated a basic artificial resin substituted by alkyl radicals. 50

14. An article as defined in claim 10, in which the alkyl radicals are methyl groups. 55

60 PAUL SCHLACK.